

May 20, 1952

V. C. CAMPBELL

2,597,617

METHOD OF DEPOSITING AN IMPERVIOUS METAL  
FILM ON A GRANULAR SURFACE

Filed Nov. 9, 1946



Fig. 2.



Fig. 3.



Fig. 4.



Inventor:  
Von C. Campbell,

by Merton D. Moore  
His Attorney.

## UNITED STATES PATENT OFFICE

2,597,617

METHOD OF DEPOSITING AN IMPERVIOUS  
METAL FILM ON A GRANULAR SURFACE

Von C. Campbell, Scotia, N. Y., assigner to General Electric Company, a corporation of New York

Application November 9, 1946, Serial No. 709,037

2 Claims. (Cl. 117—33.5)

1

My invention relates to an improved method of depositing a smooth film on a granular surface and specifically to an improved method of applying an impervious metal film on the fluorescent screen of a cathode ray tube.

In the operation of cathode ray tubes in television receivers, considerable difficulty is encountered as a result of darkening or burning of the fluorescent screen by ions which are present in the electron beam. It is known that this difficulty may be avoided by applying a thin, impervious metal backing over the fluorescent screen. Known methods for applying coatings of this type have not been well adapted for factory production and have failed to produce a thin coating which is sufficiently free from perforations. The present invention provides a method which overcomes both of these defects.

It is an object of my invention to provide an improved method of depositing a smooth film on a granular surface.

It is another object of my invention to provide an improved method of applying a thin conducting coating on the fluorescent screen of a cathode ray tube.

Further objects and advantages of my invention will become apparent as the following description proceeds, reference being had to the accompanying drawing, and its scope will be pointed out in the appended claims. In the drawing Fig. 1 is an elevational view partially in section of a cathode ray tube embodying my invention and Figs. 2 to 4 inclusive are enlarged views in section illustrating various steps in a process embodying my invention.

Referring now to the drawing, there is illustrated in Fig. 1 a cathode ray tube of a type to which my invention may be applied with particular advantage. The tube as illustrated includes an envelope having an enlarged bulbous portion 1 and an elongated shaft portion 2. The latter portion contains an electron gun 3 for generating an electron beam adapted to be projected longitudinally of the envelope. A conducting coating 4 which may, for example, be an aqueous suspension of graphite, is applied to the inner surface of the envelope. As illustrated in the drawing, the coating may extend from the large end of the envelope substantially to the electron gun and provides an accelerating electrode by means of which an appropriate axial electric field may be produced within the envelope. The large end of the envelope provides a transparent window 5 which is provided on its inner surface with a layer 6 of a fluorescent ma-

2

terial which is adapted to be excited to visible luminescence by the impingement of electrons. Suitable electron deflecting means illustrated diagrammatically as electromagnetic deflecting coils 5 7 and 8 are provided for the purpose of causing the electron beam to scan elemental areas of the screen to develop a picture thereon.

In the operation of tubes of the type just described, a dark spot tends to form on the center portion of the fluorescent screen. The darkening in the screen has been attributed to the presence of ions in the electron beam which are not deflected by the electromagnetic deflecting means and which tend to burn the fluorescent material. These ions may be prevented from producing this detrimental effect by providing a metal film on the back of the fluorescent material. This film if imperforate and thin permits the electrons to pass through to the screen substantially unimpeded while collecting substantially all of the ions. A conducting backing also eliminates a tendency for charges to accumulate on the screen and to minimize the projection of light from the screen to the interior of the tube envelope.

In accordance with my invention, the metal backing which may be of such materials as aluminum or beryllium is applied to the granular fluorescent coating by the successive steps illustrated in Figs. 2 to 4 inclusive. In Fig. 2 an enlarged section of the window of the tube is illustrated at 5 and the granular structure of the fluorescent screen is designated by the numeral 6'. In the first step of the process a controlled amount of liquid is applied to the fluorescent screen so that the interstices are just filled with the liquid as illustrated at 9. While a number of liquids may be employed, I have found that water is particularly suitable. The amount 30 of water may be controlled by applying a measured quantity to a tube of given dimensions or as I have found preferable an excess of water may be introduced into the interior of the tube and flushed over the fluorescent screen. The 40 tube envelope may then be inverted and the excess water drained off. The removal of the excess may be accelerated by the application of heat if desired. Some experimentation is required with tubes of different sizes and with 50 screens having different granular screen structures to determine the exact technique required to provide just enough liquid on the screen to fill the interstices.

The next step of the process is accomplished 55 by flowing over the surface provided by the

screen and water, a very thin layer of a film-forming resin dissolved in a volatile solvent. A large number of synthetic resins are suitable for this purpose, and I have found that a resin produced by the reaction of an aldehyde with a hydrolyzed polymerized vinyl ester is particularly suitable for this process. The resin which is insoluble in water is dissolved in a suitable solvent which may, for example, be ethylene dichloride. The solution is flushed over the surface to provide a thin film, for example, 500 to 10,000 angstrom units, and the film allowed to set (by evaporation of the solvent). The surface of the resin layer 10 thus applied is very smooth and provides a suitable carrier on which the metal backing may be deposited. The metal may be deposited on the resin film by a suitable evaporation process to provide a thin layer of suitable thickness as designated in Fig. 4 by numeral 11. The metal film produced is of uniform thickness and relatively free from small holes. In the completion of the tube the screen is heated to a relatively high temperature, for example, in the order of 400° C. This heating removes any residual moisture and also removes substantially all the resin film, leaving the thin metallic coating over the back of the screen. This heating may be performed in air or vacuum. Baking out in vacuum yields films of excellent reflectivity. Air baking decreases the reflectivity somewhat, probably about 20 per cent reduction.

The method described above in connection with the manufacture of cathode ray tubes for television purposes may be applied to the coating of other granular materials with a thin impervious metal coating. When used for television tubes the metal films improve contrast very considerably as light output is increased and no back lighting results.

While I have described and illustrated a particular embodiment of my invention, it will be obvious to those skilled in the art that changes and modifications may be made without departing from my invention in its broader aspects and I therefore, aim in the appended claims to cover all such changes and modifications as fall within the true spirit and scope of my invention.

What I claim as new and desire to secure by Letters Patent of the United States is:

1. The method of producing a smooth thin metal backing on a granular fluorescent screen which comprises the steps of applying sufficient water to the screen to fill the intergranular spaces, covering the screen and water with a layer of a solution of water-insoluble synthetic heat removable resin in a volatile non-aqueous solvent to a thickness in the order of 500 to 10,000 angstrom units, evaporating the solvent to cause the resin to set, depositing a thin layer of metal on the resin by vaporizing the metal and baking the screen at a temperature in the order of 400° C. to remove the resin and complete the metal backed fluorescent screen.

2. The method of producing a smooth thin metal backing on a granular fluorescent screen which comprises the steps of applying sufficient water to the screen to fill the intergranular surface, covering the screen and water with a layer of a solution of a water-insoluble synthetic heat removable resin in a volatile non-aqueous solvent to a thickness in the order of 500 to 10,000 angstrom units, said resin being the reaction product of an aldehyde with a hydrolyzed polymerized vinyl ester, allowing the resin to set by vaporization of the solvent, depositing a thin layer of metal on the resin by vaporizing the metal on the resin layer and baking the screen to a temperature in the order of 400° C. to remove the resin and complete the metal backed fluorescent screen.

VON C. CAMPBELL.

#### REFERENCES CITED

The following references are of record in the file of this patent:

#### UNITED STATES PATENTS

| Number    | Name      | Date          |
|-----------|-----------|---------------|
| 2,233,736 | Law       | Mar. 4, 1941  |
| 2,285,424 | Fenner    | June 9, 1942  |
| 2,373,849 | Palmer    | Apr. 17, 1945 |
| 2,374,310 | Schaeffer | Apr. 24, 1945 |
| 2,400,304 | Hamel     | May 14, 1946  |